

UNITED STATES PATENT OFFICE

2,336,463

# CYANINE DYE CONTAINING A TETRAHYDROBENZOTHIAZOLE NUCLEUS

Leslie G. S. Brooker and Frank L. White, Rochester, N. Y., assignors to Eastman Kodak Company, Rochester, N. Y., a corporation of New Jersey

No Drawing. Application November 9, 1939,  
Serial No. 303,618

4 Claims. (Cl. 260—240)

This invention relates to cyanine dyes containing a tetrahydrobenzothiazole nucleus and to a process for preparing such dyes.

Cyanine dyes contain at least two auxochromic nitrogen atoms, the one ternary and the other quaternary, the one nitrogen atom lying in one heterocyclic nucleus and the other lying in another heterocyclic nucleus, the two nitrogen atoms being connected by a conjugated carbon chain. A number of cyanine dyes containing benzothiazole nuclei as one or both of the aforementioned heterocyclic nuclei are known.

We have now found that it is possible to prepare cyanine dyes in which one or both of the aforesaid auxochromic nitrogen atoms lie in a 4,5,6,7-tetrahydrobenzothiazole nucleus. We have further found that these new cyanine dyes sensitize photographic emulsions strongly and cleanly, i. e. without producing excessive fog.

It is, accordingly, an object of our invention to provide new cyanine dyes. A further object is to provide a method for preparing such dyes. A further object is to provide photographic emulsions sensitized with such dyes. Other objects will appear hereinafter.

As starting material for the preparation of our new dyes, we employ 2-alkyl-4,5,6,7-tetrahydrobenzothiazoles, particularly 2-methyl-4,5,6,7-tetrahydrobenzothiazole. We first convert these tetrahydrobenzothiazole bases to quaternary salts by reacting the bases with esters, such as alkyl halides, alkyl sulfates or alkyl-p-toluenesulfonates, for example.

To prepare pseudocyanine dyes from such quaternary salts, we react the quaternary salts with 2-halogenoquinoline quaternary salts, in the presence of an acid-binding agent, such, for example, as sodium ethylate, sodium carbonate, pyridine or a strong tertiary organic base (e. g. trimethylamine, triethylamine and N-methyl-piperidine). Strong organic bases are those which have a dissociation constant substantially greater than that of pyridine. We have found it advantageous to employ strong tertiary organic bases.

Instead of 2-halogenoquinoline quaternary salts, we can employ 2-alkylmercapto- or 2-arylmercaptoquinoline quaternary salts to condense with the quaternary salts of 2-alkyltetrahydrobenzothiazoles, in the presence of an acid-binding agent. 2-alkylmercapto- and 2-arylmercaptoquinoline quaternary salts are described in United States Patent 2,117,936, dated May 17, 1938.

Using 2-halogenopyridine or 2-halogenopyridine quaternary salts instead of 2-halogenoquinoline quaternary salts, we can prepare pyrido-pseudocyanine dyes containing a tetrahydrobenzothiazole nucleus.

Using 2-alkylmercapto- or 2-arylmercapto-benzothiazole quaternary salts instead of 2-halo-  
genoquinoline quaternary salts, we can prepare simple cyanine dyes other than pseudocyanine dyes.

To prepare symmetrical carbocyanine dyes from 2 - alkyl - 4,5,6,7 - tetrahydrobenzothiazole quaternary salts, we react the quaternary salts with esters of ortho- acids, e. g. ethyl orthoformate, ethyl orthoacetate, ethyl orthopropionate and ethyl orthobenzoate, in the presence of pyridine.

To prepare unsymmetrical carbocyanine dyes from 2-alkyl-4,5,6,7-tetrahydrobenzothiazole 20 quaternary salts, we react the quaternary salts with cyclammonium quaternary salts containing a  $\beta$ -arylaminovinyl group in the alpha or gamma position, i. e. in one of the so-called reactive 25 positions, in the presence of an acid binding agent, e. g. pyridine.

To prepare dicarbocyanine dyes from 2-alkyl-4,5,6,7-tetrahydrobenzothiazole quaternary salts, we react the quaternary salts with cyclammonium quaternary salts containing an  $\omega$ -aryl-aminobutadienyl group in the alpha or gamma position, in the presence of an acid-binding agent, e. g. triethylamine dissolved in ethyl or isopropyl alcohol.

The following examples will serve to demonstrate the manner of obtaining our new dyes. These examples, however, are not intended to limit our invention:

### EXAMPLE 1

40 1',3-diethyl-4,5,6,7-tetrahydrothia-2'-cyanine  
iodide



3.09 g. (1 mol.) of 2-methyl-4,5,6,7-tetrahydro-  
50 benzothiazole ethiodide and 4.1 g. (1 mol.) of 2-  
iodoquinoline ethiodide were mixed together in  
15 cc. of absolute ethyl alcohol. The resulting  
mixture was heated to boiling under reflux, when  
2.1 g. (2.1 mol.) of triethylamine were added  
55 gradually to the refluxing mixture, while agitat-

ing the mixture. Boiling was continued for about 20 minutes. At the end of this time, the reaction mixture was cooled and chilled to 0° C. The dye separated from the chilled reaction mixture. The dye was filtered off, washed with acetone, then with water and finally with acetone, and then allowed to dry in the air. A yield of 84% of dye was thus obtained. The crude dye was recrystallized from methyl alcohol (25 cc. per gram of dye) and a 65% yield of pure dye was obtained. The pure dye was obtained in the form of reddish-orange crystals which melted at 279° to 280° C. with decomposition.

## EXAMPLE 2

*3,3'-diethyl-4,5,6,7,4',5',6',7'-octahydrothiacarbo-cyanine iodide*



3.09 g. (2 mol.) of 2-methyl-4,5,6,7-tetrahydrobenzothiazole ethiodide and 2.2 g. (3 mol.) of ethylorthoformate were mixed together in 10 cc. of dry pyridine. The resulting mixture was gently boiled, under reflux, for about 2 1/4 hours. At the end of this time, the reaction mixture was cooled and diethyl ether was added to the reaction mixture to precipitate the dye. The precipitated dye was filtered off, washed with water and then with acetone, and finally allowed to dry in the air. The yield of crude dye was 12%. The crude dye was recrystallized from acetone (110 cc. per gram of dye) and an 8% yield of pure dye was obtained in the form of greenish-bronze crystals melting at 216° to 217° C. with decomposition.

## EXAMPLE 3

*3,3'-diethyl-9-methyl-4,5,6,7,4',5',6',7'-octahydrothiacarbo-cyanine iodide*



3.09 g. (2 mol.) of 2-methyl-4,5,6,7-tetrahydrobenzothiazole ethiodide and 2.4 g. (3 mol.) of ethyl orthoacetate were mixed together in 10 cc. of dry pyridine. The resulting mixture was gently boiled, under reflux, for about 2 1/4 hours. The reaction mixture was then cooled and diluted with 150 cc. of diethyl ether to precipitate the dye. The ethereal layer was then decanted. The sticky residue was stirred with another 150 cc. portion of diethyl ether and again the ethereal layer was decanted. The sticky residue was dissolved in 25 cc. of acetone and the resulting solution was diluted with diethyl ether to precipitate the dye. The precipitated dye was filtered off and washed with acetone and allowed to dry in the air. The yield of crude dye was 10%. After recrystallization from acetone (160 cc. per gram of dye) a yield of 6% of pure dye was obtained. The dye was obtained in the form of dull dark green crystals, melting at 246° to 248° C. with decomposition.

## EXAMPLE 4

*3,3',9-triethyl-4,5,6,7,4',5',6',7'-octahydrothiacarbo-cyanine iodide*



7.06 g. (2 mol.) of 2-methyl-4,5,6,7-tetrahydrobenzothiazole etho-p-toluenesulfonate and 5.28 g. (3 mol.) of ethyl orthopropionate were mixed together in 10 cc. of dry pyridine. The resulting mixture was gently boiled, under reflux, for about 4 hours. At the end of this time, the hot reaction mixture was treated with a hot solution of potassium iodide (5 g.) dissolved in water (50 cc.). The resulting mixture was chilled to 0° C. when the dye separated out. It was filtered off, washed with water and finally stirred with boiling acetone (25 cc.). The acetone suspension was chilled to 0° C. and the dye filtered off and washed with cold acetone and allowed to dry in the air. The yield of crude dye was 16% and after two recrystallizations from acetone (100 cc. per gram of dye), a yield of pure dye of 7% was obtained. The dye was obtained in the form of dark green crystals.

## EXAMPLE 5

*3,3'-diethyl-4',5',6',7'-tetrahydro-oxathiacarbo-cyanine iodide*



3.53 g. (1.1 mol.) of 2-methyl-4,5,6,7-tetrahydrobenzothiazole etho-p-toluenesulfonate and 3.95 g. (1 mol.) of 2-( $\beta$ -acetanilidovinyl)-benzoxazole ethiodide were mixed together in 15 cc. of dry pyridine. The resulting mixture was gently boiled, under reflux, for about 10 minutes. The reaction mixture was then cooled and diluted with 150 cc. of diethyl ether. The ethereal layer was decanted and the residue was stirred with 50 cc. of hot acetone. The resulting acetone suspension was chilled to 0° C. and the dye was filtered off and washed with cold acetone. The dye was allowed to dry in the air. The yield of crude dye was 45% and after two recrystallizations from methyl alcohol (45 cc. per gram of dye), a 26% yield of pure dye was obtained. The pure dye was obtained in the form of dark purple crystals having a blue reflex and melting at 217° to 248° C. with decomposition.

## EXAMPLE 6

*3-ethyl-3'-methyl-4',5',6',7'-tetrahydrothia-carbo-cyanine iodide*



4.42 g. (1.3 mol.) of 2-methyl-4,5,6,7-tetrahydrobenzothiazole metho-p-toluenesulfonate and 4.5 g. (1 mol.) of 2-( $\beta$ -acetanilidovinyl)-benzothiazole ethiodide were mixed together in 15 cc. of dry pyridine. The resulting mixture was gently boiled, under reflux, for about 10 minutes. The reaction mixture was then chilled and the crystalline dye which separated was filtered off, washed with acetone and allowed to dry in the air. The yield of crude dye was 62% and after recrystallization from methyl alcohol (75 cc. per gram of dye), a yield of pure dye of 42% was obtained. The pure dye was in the form of dark green needles having a blue reflex and melting at 273° to 274° C. with decomposition.

## EXAMPLE 7

## Neocarbocyanine perchlorate from 2-methyl-4,5,6,7-tetrahydrobenzothiazole



7.06 g. (3 mol.) of 2-methyl-4,5,6,7-tetrahydrobenzothiazole etho-p-toluenesulfonate and 4.44 g. (1 mol.) of ethyl orthoformate were mixed together in 10 cc. of dry pyridine. The resulting mixture was gently boiled, under reflux, for about 4 hours. The hot reaction mixture was then treated with a hot solution of potassium iodide (5 g.) in water (50 cc.) and the resulting mixture was chilled at 0° C. The dye which separated was filtered off and washed with water. The dye was then stirred with 25 cc. of hot acetone. The resulting suspension was chilled to 0° C. and the dye filtered off and washed with cool acetone. The yield of crude dye-iodide was 32%, and after two recrystallizations from 95% ethyl alcohol (25 cc. per gram of dye) a yield of pure dye of 18% was obtained. The pure dye-iodide was dissolved in hot methyl alcohol (20 cc.) and to the hot solution was added a hot solution of sodium perchlorate (1 g. in 20 cc. of water). The resulting solution was chilled to 0° C. and the dye-perchlorate was filtered off. It was recrystallized from 95% ethyl alcohol (70 cc. per gram of dye) and obtained as shiny green crystals, melting at 244° to 246° C. with decomposition.

2-alkyl-4,5,6,7-tetrahydrobenzothiazoles can be prepared as described by Smith and Sapiro in *Transactions of the Royal Society of South Africa*, vol. 18, pages 229-235, 1929.

Quaternary salts of 2-alkyl-4,5,6,7-tetrahydrobenzothiazoles can be prepared as illustrated in the following examples:

## EXAMPLE 8

## 2-methyl-4,5,6,7-tetrahydrobenzothiazole ethiodide

1.53 g. of 2-methyl-4,5,6,7-tetrahydrobenzo-

thiazole and 2.0 g. of ethyl iodide were heated together, under reflux, for about 24 hours. The solid reaction product consists essentially of the quaternary salt and can be used without further 5 purification.

## EXAMPLE 9

## 2-methyl-4,5,6,7-tetrahydrobenzothiazole etho-p-toluenesulfonate

10

3.06 g. of 2-methyl-4,5,6,7-tetrahydrobenzothiazole and 4.0 g. of ethyl-p-toluenesulfonate were heated together at 100° C. for four days.

15 The solid reaction product consists essentially of the quaternary salt and can be used without further purification. The metho-p-toluenesulfonate can be similarly formed by using methyl instead of ethyl-p-toluenesulfonate.

20 To sensitize photographic silver halide emulsions with our new dyes, we disperse the dyes in the emulsions. Our invention is particularly directed to the customarily employed gelatino-silver-halide emulsions, such as the gelatino-silver-bromide, bromide and chloro-bromide for example. The methods of incorporating dyes in emulsions are simple and well known to those skilled in the art. In practicing our invention, it is convenient to add the dyes 25 from solutions in appropriate solvents. Methanol has proven satisfactory as a solvent for our new dyes. The dyes are advantageously incorporated in the finished, washed emulsions and should be uniformly distributed throughout to secure best 30 results.

35 The concentration of our new dyes in the emulsions can vary widely, e. g. from about 5 to about 100 mg. per liter of flowable emulsion. The concentration of the dye will vary according to the 40 type of light-sensitive material in the emulsion and according to the effects desired. The suitable and most economical concentration for any given emulsion will be apparent to those skilled in the art, upon making the ordinary tests and 45 observations customarily used in the art of emulsion-making. To prepare a gelatino-silver-halide emulsion sensitized with one of our new dyes, the following procedure is satisfactory: A quantity of the dye is dissolved in methyl alcohol, 50 and a volume of the solution (which may be diluted with water) containing from 5 to 100 mg. of dye is slowly added to about 1000 cc. of a gelatino-silver-halide emulsion with stirring. Stirring is continued until the dye is uniformly 55 dispersed. With the more powerful of our new sensitizing dues, 10 to 20 mg. of dye per 1000 cc. of emulsion suffice to produce the maximum sensitizing effect with the ordinary gelatino-silver-halide emulsions. The above statements are 60 only illustrative and not to be understood as limiting our invention in any sense, as it will be apparent that our dyes can be incorporated by other methods in many of the photographic emulsions customarily employed in the art, such, for instance, as by bathing the plate or film upon 65 which the emulsion is coated, in a solution of the dye in an appropriate solvent, although such a method is ordinarily not to be preferred. The claims are intended to cover any combination of these new dyes with a photographic silver halide emulsion whereby the dyes exert a sensitizing 70 effect on the emulsion.

75 The following table contains data which show the sensitizing range of our new dyes on photographic silver halide emulsions:

Table

| Emulsion                                                                         | Dye (mg. per liter of emulsion)                                                           | Sensitivity<br>extends to | Maximum<br>sensitivity |
|----------------------------------------------------------------------------------|-------------------------------------------------------------------------------------------|---------------------------|------------------------|
| Gelatino-silver-bromiodide (about 40 g. of silver halide per liter of emulsion). | 1',3-diethyl-4,5,6,7-tetrahydrothia-2'-cyanine iodide. 10 mg.                             | <i>Mu</i><br>575          | <i>Mu</i><br>540       |
| Do-----                                                                          | 3,3'-diethyl-4,5,6,7,4',5',6',7'-octahydrothiacarbocyanine iodide. 10 mg.                 | 645                       | 610                    |
| Do-----                                                                          | 3,3'-diethyl-9-methyl-4,5,6,7,4',5',6',7'-octahydrothiacarbocyanine iodide. 10 mg.        | 615                       | 580                    |
| Do-----                                                                          | 3,3',9-triethyl-4,5,6,7,4',5',6',7'-octahydrothiacarbocyanine iodide. 10 mg.              | 615                       | 580                    |
| Do-----                                                                          | 3,3'-diethyl-4',5',6',7'-tetrahydro-oxathiacarbocyanine iodide. 10 mg.                    | 585                       | 580                    |
| Do-----                                                                          | 3-ethyl-3'-methyl-4',5',6',7'-tetrahydrothiacarbocyanine iodide. 10 mg.                   | 640                       | 600                    |
| Do-----                                                                          | Neothiazolocarbocyanine perchlorate from 2-methyl-4,5,6,7-tetrahydrobenzothiazole. 20 mg. | 725                       | 680                    |

Photographic elements comprising our new dyes can be prepared in the usual manner by coating the emulsions on a suitable support (e. g. glass, cellulose derivative film, resin film or photographic paper) to suitable thickness and drying the coated emulsion.

What we claim as our invention and desire to be secured by Letters Patent of the United States is:

1. A dye selected from the group characterized by the following general formula:



wherein R and R' represent alkyl groups, R'' represents a substituent selected from the group consisting of hydrogen and alkyl groups and X represents an acid radical.

2. 3,3'-diethyl-4,5,6,7,4',5',6',7'-octahydrothiacarbocyanine iodide.

3. 3,3' - diethyl-9-methyl-4,5,6,7,4',5',6',7'-octahydrothiacarbocyanine iodide.

4. 3,3',9-triethyl-4,5,6,7,4',5',6',7' - octahydrothiacarbocyanine iodide.

LESLIE G. S. BROOKER.  
FRANK L. WHITE.